

## UNITED STATES PATENT OFFICE

2,668,780

## METHOD FOR RENDERING CELLULOSIC MATERIALS FIRE RESISTANT

Irene M. Panik, Elizabeth, N. J., and William F. Sullivan, Oak Ridge, Tenn., assignors to National Lead Company, New York, N. Y., a corporation of New Jersey

No Drawing. Application November 27, 1951,  
Serial No. 258,533

4 Claims. (Cl. 117—62)

1

This invention relates to a method for rendering materials fire resistant. This is a continuation-in-part of our copending application Serial No. 229,272 filed May 31, 1951. More specifically it relates to a method for rendering cellulosic materials fire resistant.

Many types of agents have been proposed for rendering cloth, paper and other fibrous materials fire resistant, and some have been successfully employed but few have the necessary properties to be able to withstand the rigors of handling and cleaning, particularly of washing and laundering. Some of the known treating agents are capable of being washed and laundered to a limited degree, but most of them appreciably alter the appearance, texture or tensile strength of the treated cellulosic material. In addition many of the known agents are not sufficiently adherent and tend to separate from the treated material in the form of fine dust.

Among the fire retarding agents which are non-launderable are the phosphate, borate and sulfamate types. Launderable types of agents include resins, chlorinated resins, or waxes added in combination with inorganic oxides such as antimony oxide. They, however, have the disadvantage of altering the appearance of the material considerably, and that they must be added in large quantity. Titanium has been added in several fire resistant processes, but in most of these the titanium has been added as titanium dioxide in order to obtain opaque pigment effects.

Titanium tetrachloride solutions have been tried for rendering cellulosic materials fire resistant but have met with the disadvantage that the solution is too acid and therefore has undesirable tendering effects on the cellulosic materials. It is therefore necessary to employ titanium salt solutions which are not as strongly acid as titanium tetrachloride. It has been found that aqueous solutions of partially substituted chlorides of tetravalent titanium may be used for rendering cellulosic materials fire resistant without tenderizing the material. Solutions which fall within the partially substituted chlorides are basic titanium chloride solutions, that is a portion of the chloride ions replaced by hydroxyl or oxidic groups (better known and sometimes referred to hereinafter as titanium oxychlorides), and titanium organo chlorides such as e. g. titanium chloride acylate solutions. It has been found that preferably from 1 to 3 of the chloride ions may be substituted by other groups including oxidic or hydroxyl groups of organic radicals. The preparation of a titanium

2

chloride acylate solution is more particularly described and claimed in co-pending application Serial No. 229,274 filed May 31, 1951. Basic titanium chloride solutions containing small amounts of soluble phosphates are particularly desirable to employ in the process of the instant invention. These solutions are more particularly described and claimed in co-pending application Serial No. 253,973 filed October 30, 1951. In order to improve flame resistance together with resistance to afterglow it is desirable to add antimony chloride to the aqueous solution of partially substituted chloride of tetravalent titanium.

When treating cellulosic materials with these solutions according to known methods the treated material exhibits some measure of fire retardance but cannot withstand the rigors of repeated launderings. Also the appearance of the cellulosic material is changed to a dusty chalky character and the loss of the titanium values is considerable during the processing steps.

An object of this invention is to provide a process wherein cellulosic materials may be rendered fire resistant and capable of withstanding repeated washings or launderings. A further object is to provide a method for rendering cellulosic materials fire resistant which will not change the appearance or texture of such materials. A further object is to provide a method for rendering cellulosic materials fire resistant by a process which will utilize substantially all of the titanium values in said solutions. These and other objects of the present invention will become apparent as the invention is more fully described.

In its broadest aspects this invention contemplates a process for rendering cellulosic materials fire resistant by impregnating the material with an aqueous solution of partially substituted chlorides of tetravalent titanium, partially drying said solution on said material to form a transparent gel, alkalizing the gelatinized solution retained in said material with an alkaline neutralizing agent and subsequently washing and drying said material. It is desirable to impregnate said material with an amount of solution which is equivalent to form 60% to 100% of the weight of the cellulosic material. In order to form a transparent gel on the cellulosic material by the partial drying step, it has been found that from 50% to 75% of the weight of the solution impregnated in the cloth should be removed. For improved flame resistance together with improved resistance to afterglow the above process may be carried out using an aqueous solution

of partially substituted chlorides of tetravalent titanium which contains antimony chloride.

Fibrous cellulosic materials which may be rendered fire resistant by the process of the instant invention includes fabrics such as cotton, linen, regenerated cellulose, viscose and cellulose acetate, also natural fibers such as kapok, hemp, wood and wood products such as pressed boards, cardboard, batting, paper, wood flour, sawdust, and the like.

The cellulosic material may be treated with the aqueous solution of partially substituted chlorides of tetravalent titanium by any convenient means such as by dipping the material in the solution, or by spraying the solution on the material. Any excess solution on the cellulosic material may be removed, for example, by squeezing between rolls, deliquoring in a filter press or by any other appropriate methods depending upon the physical nature of the material employed.

As stated previously in the impregnation step it is preferred to leave a quantity of solution on the cellulosic material from about 60% to about equal to the weight of the material itself, i. e. a weight pick-up of about 60% to 100%.

In most prior art methods the material impregnated with the solution would be substantially immediately alkalized with an alkalizing agent (without a partial drying step), thoroughly washed and dried.

By such prior art procedures which do not include a partial drying step with this type of solutions from about 30% to 70% of the titanium values would be precipitated from solution and fall to the bottom of the neutralizing tank. The cellulosic material processed according to these well-known methods would exhibit relatively poor fire resistant characteristics and would exhibit a dusty and chalky appearance. The fire retardancy would be poor at the onset and would be diminished rapidly upon repeated washing and laundering of the cellulosic material.

By introducing the partial drying step which is essential in the process of the instant invention, superior flame resistance is obtained on the treated material. The loss of the titanium values is very small during the neutralizing step and no dusting or chalking, or change in the physical appearance of the material is apparent. Such a partial drying step should be carried out by exposing the impregnated material to the atmosphere for a short interval of time to reduce by evaporation the weight of the solution held by the cellulosic material to  $\frac{1}{2}$  to  $\frac{3}{4}$  the amount picked up or impregnated in the cellulosic material.

It has been found that the partial drying operation may be carried out at room temperature or temperatures up to 60° C. Obviously at elevated temperatures less time is necessary to partially dry this solution on the material. It has been found that 45 minutes drying time is necessary at room temperatures (temperatures under atmospheric conditions). At 40° C. 35 minutes may be employed while at 60° C. 10 minutes may be employed. During such partial drying step the solution is gelatinized on cellulosic material forming a transparent gel, and substantially all of the titanium values impregnated in the cloth are retained in this gel formation.

The cellulosic material containing the gelatinized treating agent is then subjected to an alkalizing agent in order to raise the pH of the treated material to above 7.5 preferably above 9.0 but not exceeding about 12.0. The type of alka-

lizing agent used is unimportant although weak alkalizing agents such as, for example, sodium carbonate or ammonium hydroxide or carbonate, are preferred. Small amounts of soluble silicates such as sodium silicate may be added with the neutralizing or alkalizing agent if desired. By such addition the treated cloth will possess better resistance to afterglow than treated otherwise. The amount of soluble silicate should be that required to give from 0.2 to 1.5, preferably about 1.0%  $\text{SiO}_2$  on the final treated material. Such soluble silicates may also be added to the material prior to impregnation with the solution of partially substituted chloride of tetravalent titanium; or after the neutralization step, but it is preferred to add the soluble silicate during the neutralization step. The material is then rinsed well with water, for example by decantation, in order to remove the soluble salts therefrom and subsequently dried.

It has been found that the preferred amount of impregnant on the final material (dry basis) is about 6.0% to 9.0% of the weight of the fibrous cellulosic material when the partially substituted chloride of tetravalent titanium solution is used alone, while about 14% to 16% is preferred when the solution contains antimony chloride.

The entire process may be carried out at room temperature although if desired, temperatures up to 60° C. may be employed.

The exact nature of the physical and chemical changes that take place during this process is not completely understood. However, the solution of partially substituted chloride of tetravalent titanium is apparently converted to a transparent gel during the drying operation. This transparent gel adheres tenaciously to the cellulosic material and is not removed by subsequent washing. It may be held in the pores or between the fibers of the cellulosic material, may be absorbed or adsorbed on the surface or may react to some extent with the cellulosic material itself.

To illustrate preferred embodiments of this invention, the following examples are presented:

#### EXAMPLE 1

A basic tetravalent titanium chloride solution containing 200 grams per liter antimony chloride, 60 grams per liter of titanium and 84 grams per liter of chloride in addition to the chloride values of the antimony chloride was used for treating a piece of cotton cloth. The cloth was cotton twill weighing 8.2 ounces per square yard.

The cloth was immersed in the aqueous solution of basic titanium chloride for 2½ minutes and was passed through a hand wringer. The operation was repeated a second time (immersed and wrung again) to obtain good soaking. The treated cloth was weighed and found to contain a weight pick-up of 100%, i. e. the solution retained in the cloth weighed as much as the cloth itself. The treated cloth was then partially dried by exposing the cloth to the atmosphere at room temperature for 2 hours. After the partial drying step the cloth was weighed again and it was found that the weight of the solution on the cloth had been decreased to 50% of the original weight pick-up on the cloth. During the partial drying operation the solution was gelatinized on the cloth to form a transparent gel. The gel-containing treated cloth, after the partial drying operation was then immersed for 5 minutes in a solution of sodium hydroxide containing 200 grams per liter NaOH to alkalize the solution retained on the cloth. The pH of the retained

solution held by the cloth was 9.5. The excess solution was squeezed out of the cloth by passing the cloth through a hand wringer. The cloth was then washed well with water until the retained solution had a pH of 8.0. The washed cloth was then thoroughly dried. The entire procedure was carried out at room temperature. The treated cloth was subjected to a standard flame test and the results are recorded in Table 1.

The standard flame test is called the 45° Micro-burner test and consists of exposing the smooth side of the fabric at an angle of 45°  $\frac{3}{4}$  inch above the top of a burner. The flame,  $1\frac{1}{4}$  inches in length, is played onto the fabric for 12 seconds. The afterflaming and afterglow data are recorded in seconds. The procedure and apparatus assembly has been developed by the Quarter-

10

15

5 A basic tetravalent titanium chloride solution containing soluble phosphate was used in this example for treating a cotton cloth. This solution was prepared by the method described in co-pending application Serial No. 253,973. Again the procedure described in Example 1 was em-

ployed except that the weight pick-up was 70% and it was partially dried until one-half of the weight pick-up had been removed. The solution was partially dried on the cloth by exposing to

the atmosphere at 40° for 35 minutes. The results along with the control run are again re-

corded in Table 1.

Table 1

|                                                                  | Example 1<br>Basic titanium chloride<br>and antimony chloride |                          | Example 2<br>Titanium chloride acetate  |                        | Example 3<br>Basic titanium chloride con-<br>taining soluble phosphates |                        |
|------------------------------------------------------------------|---------------------------------------------------------------|--------------------------|-----------------------------------------|------------------------|-------------------------------------------------------------------------|------------------------|
|                                                                  | Partial<br>Drying<br>Step In-<br>cluded in<br>Process         | Not Par-<br>tially Dried | Partial<br>Drying<br>Step In-<br>cluded | Not Partially<br>Dried | Partial<br>Drying<br>Step In-<br>cluded                                 | Not Partially<br>Dried |
| Afterflame (sec.)                                                | 0.....                                                        | 18.....                  | 8.....                                  | completely burned      | 10.....                                                                 | completely burned.     |
| Appearance                                                       | not dusty.                                                    | dusty.....               | not dusty.....                          | dusty.....             | not dusty.....                                                          | dusty.                 |
| Percent Titanium Values<br>Lost During Neutraliza-<br>tion Step. | 0.....                                                        | 50.....                  | 0.....                                  | 40.....                | 0.....                                                                  | 60.                    |

master Corps of the United States Army and is described by Robert W. Little, Major in Quarter- 35 master Corps, in his book entitled "Flameproofing Textile Fabrics" on pages 117-119, Reinhold Publishing Corporation, 1947.

In order to compare the process of the instant invention with a process in which the partial drying step has been omitted the following description is presented:

Another piece of cloth of the type previously described was placed in the same basic titanium chloride solution until substantially 100% weight pick-up was obtained. Within a few minutes after the immersion step had been completed, the impregnated cloth was neutralized without the partial drying step. Again the cloth was neutralized by immersing for 5 minutes in a solution of sodium hydroxide as described above. The neutralized cloth was then processed according to the above procedure. The cloth was then subjected to the standard flame test and the results are recorded in Table 1.

## EXAMPLE 2

A titanium chloride acetate solution containing 77 grams per liter of titanium, 262 grams per liter of acetate and 70 grams per liter chloride was diluted with water to produce a solution containing 60 grams per liter titanium. Such a solution was prepared by the method described in co-pending application Serial Number 229,272 filed May 31, 1951.

The procedure described in Example 1 was repeated using this titanium chloride acetate solution except the partial drying step was carried out at a temperature of 50° C. and the drying time was 15 minutes. The results of the standard flame test on the treated cloth are recorded in Table 1.

Again in order to show a comparison between the process of the instant invention with a procedure which does not utilize a drying step, a cloth was treated in the same solution in the

5 It should be noted that the data presented in Table 1 shows the results after laundering. The laundering process was carried out in a tumbling chamber with 0.5% soap solution at 75° C.

While the examples illustrate the employment of titanium chloride acetate solution, this being 40 the preferred titanium chloride acylate, solutions of titanium chloride formate and titanium chloride propionate may be employed with similar effect. These compounds, however, are somewhat more expensive to produce and therefore not as economical as the acetate salt.

45 By the utilization of the process of this invention which includes the partial drying step, it has clearly been shown that the titanium values are fixed in the material in a form in which substantially no alteration in appearance or texture of the material is observed. It should be noted that by applying the process of the instant invention increased flame resistance is obtained with substantially no loss of the titanium and antimony values during processing. The process is economical to employ and simple to operate and decided improvements are obtained in the

50 appearance, texture of the treated fabric in the flame resistant characteristics and in the utilization of substantially all of the titanium and antimony values.

55 While this invention has been described and illustrated by the examples shown, it is not intended to be strictly limited thereto and other modifications and variations may be employed within the scope of the following claims.

We claim:

1. Method for imparting fire resistance to fibrous cellulosic material which comprises impregnating said material with a transparent aqueous solution of a substance selected from the group consisting of titanium oxychlorides, titanium chloride acylates selected from the group consisting of titanium chloride formate, titanium chloride acetate and titanium chloride propionate, and mixtures thereof, partially dry-

same manner as that described in the control run in Example 1. The results are recorded in Table 1.

## EXAMPLE 3

ing the impregnated material by evaporation until from 50% to 75% of the weight of said solution in said material is removed, thereby forming a transparent gel, alkalizing said gel in said material with an aqueous alkaline solution, and washing and drying said material, the resulting titanium substance being retained in said material in the form of a wash-fast, stable, transparent gel-like structure.

2. Method according to claim 1 wherein said transparent aqueous solution is a solution of titanium chloride acetate.

3. Method according to claim 1 wherein said transparent aqueous solution further comprises antimony chloride.

4. Method according to claim 1 wherein from

6 to 16% of said impregnated titanium substance, based on the weight of the fibrous cellulosic material, is retained in said material after washing and drying.

IRENE M. PANIK.  
WILLIAM F. SULLIVAN.

## References Cited in the file of this patent

## UNITED STATES PATENTS

|           |             |              |
|-----------|-------------|--------------|
| Number    | Name        | Date         |
| 2,570,566 | Lane et al. | Oct. 9, 1951 |

## OTHER REFERENCES

American Dyestuff Reporter, vol. 39, No. 16, Titanium Compounds as Fire Resistant Agents for Fabrics, I. M. Panik et al., Aug. 7, 1950.